

# UNITED STATES PATENT OFFICE.

LESTER KIRSCHBRAUN, OF EVANSTON, ILLINOIS, ASSIGNOR TO THE RAYBESTOS COMPANY, OF BRIDGEPORT, CONNECTICUT, A CORPORATION OF CONNECTICUT.

## FRICITION-FACING AND PROCESS OF MAKING SAME.

1,275,043.

Specification of Letters Patent. Patented Aug. 6, 1918.

No Drawing.

Application filed May 27, 1918. Serial No. 236,957.

*To all whom it may concern:*

Be it known that I, LESTER KIRSCHBRAUN, a citizen of the United States, residing in the city of Evanston, county of Cook, and 5 State of Illinois, have invented certain new and useful Improvements in Friction-Facings and Processes of Making Same, of which the following is a specification.

This invention relates to improvements in 10 friction facings and process of making same, and refers more particularly to a friction facing adapted for use in motor cars and the like.

Among the salient objects of the invention 15 are to provide a product which in its entirety is or can be made of substantially incombustible materials, at least, incombustible at temperatures to which clutch facings, brake linings and the like are subjected in use; to provide a process in which the friction facing can be formed into an 20 unwoven felted sheet made from relatively short asbestos fiber to which strength or body is given by the addition of a substantially 25 incombustible material; to provide a process in which the asbestos fiber is saturated and impregnated with a bituminous or hydrocarbon binder prior to the felting operation; to provide a process in which the 30 binder is incorporated into the asbestos at or before the felting operation; to provide a process which can be carried out as a cold 35 process and which eliminates the necessity of the use of expensive vehicles in the saturating operation, and in effect eliminates an independent saturating operation altogether; to provide a process which permits of the use of high melting point binders which are more refractory and cementitious 40 than the binders now in use for this purpose and in general to provide an improved process and product of the character described.

I am aware that heretofore there has been 45 invented an unwoven friction facing made from short asbestos fiber but as far as I know this short asbestos fiber has never theretofore been saturated or incorporated with the binder during the pulping operation or prior to the felting.

Describing now the improved product and process of making the same, I first make

an emulsion of a bituminous binder and an emulsifying agent, preferably colloidal clay, starch, cheap glue, casein or cheap 55 soap. The advantage however, of using colloidal clay or other inorganic colloidal material is that it is inexpensive and incombustible. The clay or other filler which is used as an emulsifying agent is made into 60 an aqueous paste and then melted bitumen or hydrocarbon is gradually added and stirred into the filler until a homogeneous composition results. While the hydrocarbon is being gradually added to the aqueous 65 paste hot water is also preferably added from time to time to maintain the desired working consistency. This emulsified composition thinned to the desired consistency by the addition of water is mixed with the 70 short asbestos fiber either before or after the latter is pulped. The mass is mixed together until the filler and binder have become thoroughly amalgamated with the asbestos fiber. By adding the binder to this 75 compound the asbestos fibers become thoroughly coated with the binder. The pulped mass may have more water added to it or the excess water removed from it as condition may require to produce the desired 80 working consistency, and the material is now ready for felting.

Ordinarily, in the felting operation of fibers, they are held together by a mechanical bond due to the interlacing of the fibers. 85 In the felting mixture heretofore described however, the fibers are already coated with a bituminous binder so in felting this mixture you not only get a mechanical bond due to the interlacing of the fibers but an additional bond due to the adhesion of the bituminous binder coating of the individual fibers. In the felting operation the particles of clay, if clay is used as a filler, are forced into and fill the voids between the 90 fibers and thereby add density, body and strength or toughness to the sheet.

After the felting operation, the sheet may be passed over steam heated rolls so as to drive the water out or if desired may 100 be put into a drying room to eliminate the moisture. The removal of the water or moisture from the bitumen transforms it from the state of an emulsion to that of a

homogeneous continuous binder. This material either before or after the friction facings are cut out can be run through rolls to meet the necessary micrometer measurements.

I claim as my invention:

1. A friction facing, the essential wearing surface of which consists of asbestos fiber, a colloidal filler and a binder.
- 10 2. A friction facing the wearing surface of which consists of an incombustible fiber, a bituminous binder and a relatively incom-

bustible filler, the filler and binder being in colloidal relation to each other.

3. The process of making a friction facing consisting in emulsifying a filler and a bitumen to form an emulsified composition, mixing said composition with an incombustible fiber and intimately commingling said fiber with said composition to form said last mentioned mixture into a felted unwoven sheet and drying the same to remove any moisture therefrom.

LESTER KIRSCHBRAUN.